# EUROPEAN PATENT SPECIFICATION

(11) **EP 1 774 095 B1**
(45) Date of publication and mention of the grant of the patent: **15.04.2009**
(21) Application number: 05766040.9
(22) Date of filing: 16.06.2005
(51) Int. Cl.: D21H 13/18, D21H 13/26

(54) **ACRYLIC AND PARA-ARAMID PULP AND PROCESSES OF MAKING SAME**
ACRYL- UND PARAARAMID-PULPE UND VERFAHREN ZU DEREN HERSTELLUNG
PATE A BASE DE FIBRES ACRYLIQUES ET PARA-ARAMIDES ET PROCEDES DE FABRICATION DE CETTE DERNIERE

(30) Priority: 25.06.2004 US 877843
(43) Date of publication of application: 18.04.2007
(73) Proprietor: E.I. DU PONT DE NEMOURS AND COMPANY, Wilmington, DE 19898 (US)
(72) Inventor: CONLEY, Jill, A., Midlothian, VA 23112 (US); MERRIMAN, Edmund, A., Midlothian, VA 23113 (US)
(74) Representative: Heinemann, Monica
(86) International application number: PCT/US2005/021342
(87) International publication number: WO 2006/012040

(56) References cited:
- US-A- 3 869 430
- US-A- 4 472 241
- US-A- 5 084 136
- US-A- 5 811 042
- DATABASE WPI Section Ch, Week 199812 Derwent Publications Ltd., London, GB; Class A88, AN 1998-126426 XP002353628 & JP 10 008036 A (AKEBONO BRAKE IND CO LTD) 13 January 1998 (1998-01-13)

## Description

### BACKGROUND OF THE INVENTION

### 1. Field of the Invention.

This invention relates to acrylic and para-aramid pulp for use as reinforcement material in products, such as seals and friction materials. The invention further relates to processes for making such pulp.

### 2. Description of Related Art.

Fibrous and non fibrous reinforcement materials have been used for many years in friction products, sealing products and other plastic or rubber products. Such reinforcement materials typically must exhibit high wear and heat resistance.

Asbestos fibers have historically been used as reinforcement materials, but due to their health risks, replacements have been made or proposed. However, many of these replacements do not perform as well as asbestos in one way or another.

Research Disclosure 19037, pages 74-75, published February 1980, discloses the manufacture of pulp made from fibrillated KEVLAR^{®} brand para-aramid fibers of variable lengths and use of such pulp as a reinforcement material in various applications. This publication discloses that pulp mad from KEVLAR^{®} brand para-aramid fibers can be used in sheet products alone, or in combination with fibers of other materials, such as NOMEX^{®} brand meta-aramid, wood pulp, cotton and other natural cellulosics, rayon, polyester, polyolefin, nylon, polytetrafluoroethylene, asbestos and other minerals, fiberglass and other, ceramics, steel and other metals, and carbon. The publication also discloses the use of pulp from KEVLAR^{®} brand para-aramid fiber alone, or with KEVLAR^{®} brand para-aramid short staple, in friction materials to replace a fraction of the asbestos volume, with the remainder of the asbestos volume being replaced by fillers or other fibers.

U.S. Patent 5,811,042 (to Hoiness) discloses a composite friction or gasketing material made of a thermoset or thermoplastic matrix resin, fiber reinforcing material, and substantially fibril free aramid particles. Poly (p-phenylene terephthalamide) and poly(m-phenylene isophthalamide) are preferred fiber reinforcing materials, and the fibers can be in the form of floc or pulp.

U.S. Patent Application 2003/0022961 (to Kusaka et al.) discloses friction materials made from a friction modifier, a binder and a fibrous reinforcement made of a mixture of (a) a dry aramid pulp and (b) wet aramid pulp, wood pulp or acrylic pulp. Dry aramid pulp is defined as an aramid pulp obtained by "the dry fibrillation method". The dry fibrillation method is dry milling the aramid fibers between a rotary cutter and a screen to prepare the pulp. Wet aramid pulp is defined as an aramid pulp obtained by "the wet fibrillation method". The wet fibrillation method is milling short aramid fibers in water between two rotary discs to form fibrillated fibers and then dehydrating the fibrillated fibers, i.e., the pulp. Kusaka et al further disclose a method of mix-fibrillating fibers by first mixing plural types of organic fibers that fibrillate at a definite ratio, and then fibrillating the mixture to produce a pulp.

JP 10 008036 A discloses the use of a composition of fiber base material, thermosetting resin binding material and a filler as a principle component, wherein the fiber base material contains an aramid pulp, acryl pulp, cellulose fiber, sepiolid fiber and glass fiber, for the preparation of a friction material with reduced generation of noise.

There is an ongoing need to provide alternative reinforcing materials that both perform well in products, such as seals and friction applications, and that are low in cost. Despite the numerous disclosures proposing lower cost alternative reinforcement materials, many of these proposed products do not adequately perform in use, cost significantly more than currently commercial products, or have other negative attributes. As such, there remains a need for reinforcement materials that exhibit high wear and heat resistance, and that are comparable or less expensive than other commercially available reinforcement materials.

### BRIEF SUMMARY OF THE INVENTION

The invention relates to a first embodiment of a process for making an acrylic and para-aramid pulp for use as reinforcement material, comprising:
(a) combining pulp ingredients including:
   (1) acrylic fiber comprising acrylonitrile units which are at least 85 wt % of the total acrylic fiber, the fiber being 10 to 90 wt % of the total solids in the ingredients, and having an average length of no more than 10 cm;
   (2) para-aramid fiber being 10 to 90 wt % of the total solids in the ingredients, and having an average length of no more than 10 cm; and
   (3) water being 95 to 99 wt % of the total ingredients;
(b) mixing the ingredients to a substantially uniform slurry;
(c) co-refining the slurry by simultaneously:
   (1) fibrillating, cutting and masticating the acrylic fiber and the para-aramid fiber to irregularly shaped fibrillated fibrous structures with stalks and fibrils; and
   (2) substantially uniformly dispersing all solids in the refined slurry; and
(d) removing water from the refined slurry to no more than 60 total wt % water,
thereby producing an acrylic and para-aramid pulp with the acrylic and the para-aramid fibrous structures having an average maximum dimension of no more than 5 mm, a length-weighted average of no more than 1.3 mm, and the acrylic fibrils and/or stalks are substantially entangled with the para-aramid fibrils and/or stalks.

The invention is further related to a second embodiment of a process for making an acrylic and para-aramid pulp for use as reinforcement material, comprising:
(a) combining ingredients including water and a first fiber from the group consisting of:
   (1) acrylic fiber comprising acrylonitrile units which are at least 85 wt % of the total acrylic fiber, the fiber being 10 to 90 wt % of the total solids in the ingredients; and
   (2) para-aramid fiber being 10 to 90 wt % of the total solids in the ingredients;
(b) mixing the ingredients to a substantially uniform suspension;
(c) refining the suspension in a disc refiner thereby cutting the fiber to have an average length of no more than 10 cm, and fibrillating and masticating at least some of the fiber to irregularly shaped fibrillated fibrous structures;
(d) combining ingredients including the refined suspension, the second fiber of the group of (a)(1 and 2), and water, if necessary, to increase the water concentration to 95 -99 wt % of the total ingredients;
(e) mixing the ingredients, if necessary, to form a substantially uniform suspension;
(d) co-refining the mixed suspension by:
   (1) fibrillating, cutting and masticating solids in the suspension such that all or substantially all of the acrylic and para-aramid fiber is converted to irregularly shaped fibrillated acrylic and para-aramid fibrous structures with stalks and fibrils; and
   (2) substantially uniformly dispersing all solids in the refined slurry; and
(h) removing water from the refined slurry to no more than 60 total wt % water,
thereby producing an acrylic and para-aramid pulp with the acrylic and the para-aramid fibrous structures having an average maximum dimension of no more than 5 mm, a length-weighted average of no more than 1.3 mm, and the acrylic fibrils and/or stalks are substantially entangled with the para-aramid fibrils and/or stalks.

The invention is further directed to an acrylic and para-aramid pulp for use as reinforcement material, comprising:
(a) irregularly shaped, acrylic fibrous structures comprising acrylonitrile units which are at least 85 wt % of the total acrylic fibrous structures and being 10 to 90 wt % of the total solids;
(b) irregularly shaped, para-aramid fibrous structures being 10 to 90 wt % of the total solids; and
(c) water being 4 to 60 wt % of the entire pulp,
whereby the acrylic and the para-aramid fibrous structures having an average maximum dimension of no more than 5 mm, a length-weighted average of no more than 1.3 mm, and stalks and fibrils where the acrylic fibrils and/or stalks are substantially entangled with the para-aramid fibrils and/or stalks.

The invention is further directed to a friction material, comprising a friction modifier; optionally at least one filler; a binder; and a fibrous reinforcement material comprising the pulp of the present invention.

Moreover, the invention is directed to a sealing material, comprising a binder; optionally at least one filler; and a fibrous reinforcement material comprising the pulp of the present invention.

### BRIEF DESCRIPTION OF THE DRAWING(S)

The invention can be more fully understood from the following detailed description thereof in connection with accompanying drawings described as follows.
Figure 1 is a block diagram of apparatus for performing a wet process for making "wet" pulp in accordance with the present invention.
Figure 2 is a block diagram of apparatus for performing a dry process for making "dry" pulp in accordance with the present invention.
Figure 3 is an image of a photomicrograph of para-aramid particles used as an optional ingredient to the process of the present invention.
Figure 4 is an image of a photomicrograph of pulp-made according to the process of the present invention.

### GLOSSARY

Before the invention is described, it is useful to define certain terms in the following glossary that will have the same meaning throughout this disclosure unless otherwise indicated.

"Fiber" means a relatively flexible, unit of matter having a high ratio of length to width across its cross-sectional area perpendicular to its length. Herein, the term "fiber" is used interchangeably with the term "filament" or "end". The cross section of the filaments described herein can be any shape, but are typically circular or bean shaped. Fiber spun onto a bobbin in a package is referred to as continuous fiber. Fiber can be cut into short lengths called staple fiber. Fiber can be cut into even smaller lengths called floc. Yarns, multifilament yarns or tows comprise a plurality of fibers. Yarn can be intertwined and/or twisted.

"Fibril" means a small fiber having a diameter as small as a fraction of a micrometer to a few micrometers and having a length of from about 10 to 100 micrometers. Fibrils generally extend from the main trunk of a larger fiber having a diameter of from 4 to 50 micrometers. Fibrils act as hooks or fasteners to ensnare and capture adjacent material. Some fibers fibrillate, but others do not or do not effectively fibrillate and for purposes of this definition such fibers do not fibrillate. Poly(para-phenylene terephthalamide) fiber fibrillates readily upon abrasion, creating fibrils. Acrylic fibers of this invention also fibrillate.

"Fibrillated fibrous structures" means particles of material having a stalk and fibrils extending therefrom wherein the stalk is generally columnar and about 10 to 50 micrometers in diameter and the fibrils are hair-like members only a fraction of a micron or a few microns in diameter attached to the stalk and about 10 to 100 micrometers long.

"Floc" means short lengths of fiber, shorter than staple fiber. The length of floc is about 0.5 to about 15 mm and a diameter of 4 to 50 micrometers, preferably having a length of 1 to 12 mm and a diameter of 8 to 40 micrometers. Floc that is less than about 1 mm does not add significantly to the strength of the material in which it is used. Floc or fiber that is more than about 15 mm often does not function well because the individual fibers may become entangled and cannot be adequately and uniformly distributed throughout the material or scurry. Aramid floc is made by cutting aramid fibers into short lengths without significant or any fibrillation, such as those prepared by processes described in U.S. Patent Nos. 3,063,966, 3,133,138, 3,767,756, and 3,869,430.

"Length-weighted average" means the calculated length from the following formula: $Lenght - weighted average = \frac{{\sum }_{ } \left[{\left(Each Individual pulp length\right)}^{2}\right]}{{\sum }_{ } \left[Each Individual pulp length\right]}$

"Maximum dimension" of an object means the straight distance between the two most distal points from one another in the object

"Staple fiber" can be made by cutting filaments into lengths of no more than 15 cm, preferably 3 to 15 cm; and most preferably 3 to 8 cm. The staple fiber can be straight (i.e., non crimped) or crimped to have a saw tooth shaped crimp along its length, with any crimp (or repeating bend) frequency. The fibers can be present in uncoated, or coated, or otherwise pretreated (for example, pre-stretched or heat-treated) form.

### DETAILED DESCRIPTION OF THE INVENTION

The invention is directed to processes for making an acrylic and para-aramid pulp for use as reinforcement material. The invention is also directed to acrylic and para-aramid pulp, that can be made by the processes of the invention, for use as reinforcement material. The invention is further directed to products, such as sealing materials and friction materials, incorporating the pulp of this invention, and processes for making them.

### I. First Embodiment of the Inventive Process

In a first embodiment, the process for making an acrylic and para-aramid pulp comprises the following steps. First, pulp ingredients are combined, added or contacted together. Second, the combined pulp ingredients are mixed to a substantially uniform slurry. Third, the slurry is simultaneously refined or co-refined. Fourth, water is removed from the refined slurry.

### Combining Step

In the combining step, the pulp ingredients are preferably added together in a container. The pulp ingredients include (1) acrylic fiber, (2) para-aramid fiber, (3) optionally substantially or completely fibril-free, granular, para-aramid particles, (4) optionally other minor additives, and (5) water.

### Acrylic Fiber

The acrylic fiber is added to a concentration of 10 to 90 wt % of the total solids in the ingredients, preferably 25 to 60 wt % of the total solids in the ingredients, and most preferably 25 to 55 wt % of the total solids in the ingredients.

The acrylic fiber preferably has an average length of no more than 10 cm, more preferably 0.5 to 5 cm, and most preferably 0.6 to 2 cm. Prior to combining the pulp ingredients together, any acrylic fibers in the form of continuous filaments can be cut into shorter fibers, such as staple fibers or floc.

### Acrylic Polymer

The acrylic fiber useful in this invention includes acrylonitrile units which are at least 85 wt % of the total acrylic fiber. An acrylonitrile unit is - (CH2-CHCN)-. The acrylic fiber can be made from acrylic polymers made up of 85 % by weight or more of acrylonitrile with 15 % by weight or less of an ethylenic monomer copolymerizable with acrylonitrile and mixtures of two or more of these acrylic polymers. Examples of the ethylenic monomer copolymerizable with acylonitrile include acylic acid, methacrylic acid and esters thereof (methyl acrylate, ethyl acrylate, methyl methacylate, ethyl methacrylate, etc.), vinyl acetate, vinyl chloride, vinylidene chloride, acrylamide, methacylamide, methacrylonitrile, allylsulfonic acid, methanesulfonic acid and styrenesulfonic acid.

### Para-Aramid Fiber

The para-aramid fiber is added to a concentration of 10 to 90 wt % of the total solids in the ingredients, preferably 40 to 75 wt % of the total solids in the ingredients, and most preferably 40 to 55 wt % of the total solids in the ingredients. The para-aramid fiber preferably has a linear density of no more than 10 dtex, more preferably 0.5 to 10 dtex, and most preferably, 0.8 to 2.5 dtex. The para-aramid fiber also preferably has an average length along its longitudinal axis of no more than 10 cm, more preferably an average length of 0.65 to 2.5 cm, and most preferably an average length of 0.65 to 1.25 cm.

### Para-Aramid Particles

Optionally, in one embodiment, the pulp ingredients further include substantially or completely fibril-free, granular, para-aramid particles. If these particles are added, they are added to a concentration of no more than 50 wt % of the total solids in the ingredients, preferably 20 to 50 wt % of the total solids in the ingredients, and most preferably 25 to 35 wt % of the total solids in the ingredients. Being made of para-aramid, they contribute superior wear resistance and dispersability to the pulp being produced. Because the particles are substantially fibril-free, they also serve as a compounding agent to assist in dispersing the other ingredients in the mixture and slurry. Particles that perform this function are often known as processing agents or aids. The substantially or completely fibril-free, granular, para-aramid ,particles have an average maximum dimension of 50 to 2000 micrometers (0.05 to 2 mm), preferably 50 to 1500 micrometers, and most preferably 75 to 1000 micrometers. Particles below about 50 micrometers, however, lose effectiveness in friction and sealing applications. Particles above about 2000 micrometers do not adequately stay dispersed in the water with the other ingredients when mixed. Figure 5 is an image of a photomicrograph of para-aramid particles capable of being used as an ingredient to the process of the present invention.

### Aramid Polymer

Polymers suitable for use in making the aramid fiber and aramid particles of this invention are synthetic aromatic polyamides. The polymers must be of fiber-forming molecular weight in order to be shaped into fibers. The polymers can include polyamide homopolymers, copolymers, and mixtures thereof which are predominantly aromatic, wherein at least 85% of the amide (-CONH-) linkages are attached directly to two aromatic rings. The rings can be unsubstituted or substituted. The polymers are para-aramid when the two rings are para oriented with respect to each other along the molecular chain. Preferably copolymers have no more than 10 percent of other diamines substituted for a primary diamine used in forming the polymer or no more than 10 percent of other diacid chlorides substituted for a primary diacid chloride used in forming the polymer. Additives can be used with the aramid; and it has been found that up to as much as 13 percent by weight of other polymeric material can be blended or bonded with the aramid. The preferred para-aramids are poly(para-phenylene terephthalamide)(PPD-T) and its copolymers.

### Optional Other Additives

Other additives can optionally be added as long as they stay suspended in solution in the mixing step and do not significantly change the effect of the refining step on the mandatory solid ingredients listed above. Suitable additives include pigments, dyes, anti-oxidants, flame-retardant compounds, and other processing and dispersing aids. Preferably, the pulp ingredients do not include asbestos. In other words, the resulting pulp is asbestos free or without asbestos.

### Water

Water is added to a concentration of 95 to 99 wt % of the total ingredients, and preferably 97 to 99 wt % of the total ingredients. Further, the water can be added first. Then other ingredients can be added at a rate to optimize dispersion in the water while simultaneously mixing the combined ingredients.

### Mixing Step

In the mixing step, the ingredients are mixed to a substantially uniform slurry. By "substantially uniform" is meant that random samples of the slurry contain the same wt % of the concentration of each of the starting ingredients as in the total ingredients in the combination step plus or minus 10 wt %, preferably 5 wt % and most preferably 2 wt %. For instance, if the concentration of the solids in the total mixture is 50 wt % acrylic fiber plus 50 wt % para-aramid fiber, then a substantially uniform mixture in the mixing step means each random sample of the slurry has (1) a concentration of the acrylic fiber of 50 wt % plus or minus 10 wt %, preferably 5 wt % and most preferably 2 wt % and (2) a concentration of para-aramid fiber of 50 wt % plus or minus 10 wt %, preferably 5 wt % and most preferably 2 wt %. The mixing can be accomplished in any vessel containing rotating blades or some other agitator. The mixing can occur after the ingredients are added or while the ingredients are being added or combined.

### Refining Step

In the refining step the pulp ingredients are simultaneously co-refined, converted or modified as follows. The acrylic fiber and the para-aramid fiber are fibrillated, cut and masticated to irregularly shaped fibrous structures having stalks and fibrils. If para-aramid particles are added with the other ingredients, at least some of the para-aramid particles are masticated into smaller, rounder, substantially fibril-free, particles. All solids are dispersed such that the refined slurry is substantially uniform. "substantially uniform" is as defined above. The refining step preferably comprises passing the mixed slurry through one or more disc refiner, or recycling the slurry back through a single refiner. By the term "disc refiner" is meant a refiner containing one or more pair of discs that rotate with respect to each other thereby refining ingredients by the shear action between the discs. In one suitable type of disc refiner, the slurry being refined is pumped between closely spaced circular rotor and stator discs rotatable with respect to one another. Each disc has a surface, facing the other disc, with at least partially radially extending surface grooves. A preferred disc refiner that can be used is disclosed in U.S. Patent 4,472,241. If necessary for uniform dispersion and adequate refining, the mixed slurry can be passed through the disc refiner more than once or through a series of at least two disc refiners. When the mixed slurry is refined in only one refiner, there is a tendency for the resulting slurry to be inadequately refined and non uniformly dispersed. Conglomerates or aggregates entirely or substantially of one solid ingredient, or the other, or both, or all three if three are present, can form rather than being dispersed forming a substantially uniform dispersion. Such conglomerates or aggregates have a greater tendency to be broken apart and dispersed in the slurry when the mixed slurry is passed through the refiner more than once or passed through more than one refiner.

Because a substantially uniform slurry containing multiple ingredients is co-refined in this step of the process, any one type of non-pulp ingredient (for example, para-aramid fiber) is refined into a pulp in the presence of all the other types of non-pulp ingredients (for example, aramid material pieces and optionally para-aramid particles) while those other ingredients are also being refined. This co-refining of non-pulp ingredients forms a pulp that is superior to a pulp blend generated by merely mixing two pulps together. Adding two pulps and then merely mixing them together does not form the substantially uniform, intimately connected, fibrous components of the pulp generated by co-refining of non-pulp ingredients into pulp in accordance with the present invention.

### Removing Step

Then water is removed from the refined slurry to no more than 60 total wt % water, preferably 4 to 60 total wt % water, most preferably, 5 to 58 total wt % water. The water can be removed by collecting the pulp on a dewatering device such as a horizontal filter, and if desired, additional water can be removed by applying pressure or squeezing the pulp filter cake. The dewatered pulp can optionally then be dried to a desired moisture content, and/or can be packaged or wound up on rolls.

### Figures 1 and 2

This process will now be described in reference to Figures 1 and 2. Throughout this detailed description, similar reference characters refer to similar elements in all figures of the drawings.

Referring to Figure 1, there is a block diagram of an embodiment of a wet process for making "wet" pulp in accordance with the present invention. Pulp ingredients 1 are added to container 2. Container 2 is provided with an internal mixer, similar to a mixer in a washing machine. The mixer disperses the ingredients into the water creating the substantially uniform slurry. The mixed slurry is transferred to a first refiner 3 which refines the slurry. Then, optionally, the refined slurry can be transferred to a second refiner 4, and optionally then to a third refiner 5. Three refiners are illustrated but any number of refiners can be used depending on the degree of uniformity and refining desired. After the last refiner in the series of refiners, the refined slurry is optionally transferred to a filter or sorter 6 that allows slurry with dispersed solids below a chosen mesh or screen size to pass and recirculates dispersed solids larger than a chosen mesh or screen size back to one or more of the refiners such as through line 7 or to a refiner 8 dedicated to refine this recirculated slurry from which refined slurry is again passed to the filter or sorter 6. Suitably refined slurry passes from the filter or sorter 6 to a horizontal water vacuum filter 9 which removes water such that the pulp has a concentration of water of no more than 75 wt % of the total ingredients. Slurry can be transferred from point to point by any conventional method and apparatus such as with the assistance of one or more pump 10. Then the pulp is conveyed to a dryer 11 that removes more water until the pulp has a concentration of water of no more than 60 wt % of the total ingredients. Then the refined pulp is packaged in a baler 12.

Referring to Figure 2, there is a block diagram of an embodiment of a dry process for making "dry" pulp in accordance with the present invention. This dry process is the same as the wet process except after the horizontal water vacuum filter 9. After that filter, the pulp goes through a press 13 which removes more water until the pulp has a concentration of water of no more than 20 wt % of the total ingredients. Then the pulp goes through a fluffer 14 to fluff the pulp and then a rotor 15 to remove more water. Then, like the wet process, the pulp is passed through a dryer 11 and packaged in a baler 12.

### II. Second Embodiment of the Inventive Process

In a second embodiment, the process for making the acrylic fiber and para-aramid pulp is the same as the first embodiment of the process described above with the following differences.

Prior to combining all ingredients together, either the acrylic fiber or the para-aramid fiber, or both the acrylic fiber and the para-aramid fiber, may need to be shortened. This is done by combining water with the fiber ingredient. Then the water and fiber are mixed to form a first suspension and processed through a first disc refiner to shorten the fiber. The disc refiner cuts the fiber to an average length of no more than 10 cm. The disc refiner will also partially fibrillate and partially masticate the fiber. The other fiber, that was not previously added, can be shortened this way too forming a second processed suspension. Then the other fiber (or the second suspension, if processed in water) is combined with the first suspension.

More water is added before or after, or when, other ingredients are added, if necessary, to increase the water concentration to 95 - 99 wt % of the total ingredients. After all ingredients are combined, they can be mixed, if necessary, to achieve a substantially uniform slurry.

The ingredients in the slurry are then co-refined together, i.e., simultaneously. This refining step includes fibrillating, cutting and masticating solids in the suspension such that all or substantially all of the acrylic and para-aramid fiber is converted to irregularly shaped fibrillated fibrous structures. This refining step also disperses all solids such that the refined slurry is substantially uniform. Then water is removed as in the first embodiment of the process. Both processes produce the same or substantially the same acrylic and para-aramid pulp.

### The Inventive Pulp

The resulting product produced by the process of this invention is an acrylic and para-aramid pulp for use as reinforcement material in products. The pulp comprises (a) irregularly shaped, acrylic fibrous structures, (b) irregularly shaped, para-aramid fibrous structures, (c) optionally substantially fibril-free, granular, para-aramid particles, (d) optionally other minor additives, and (e) water.

The concentration of the separate ingredient components in the pulp correspond, of course, to the concentrations described beforehand of the corresponding ingredients used in making the pulp.

The irregularly shaped, acrylic and para-aramid fibrillated fibrous structures have stalks and fibrils. The acrylic fibrils and/or stalks are substantially entangled with the para-aramid fibrils and/or stalks. The fibrils are important and act as hooks or fasteners or tentacles which adhere to and hold adjacent particles in the pulp and final product thereby providing integrity to the final product.

The acrylic and para-aramid fibrillated fibrous structures preferably have an average maximum dimension of no more than 5 mm, more preferably 0.1 to 4 mm, and most preferably 0.1 to 3 mm. The acrylic and para-aramid fibrillated fibrous structures preferably have a length-weighted average of no more than 1.3 mm, more preferably 0.7 to 1.2 mm, and most preferably 0.75 to 1.1 mm.

If para-aramid particles are included in the pulp, the acrylic and para-aramid fibrous structures also additionally contact and are wrapped partially around at least some of these rounder, substantially fibril-free, para-aramid particles. These para-aramid particle also preferably have a dimension of at least 50 micrometers, more preferably, 50 to 100 micrometers, and most preferably 50 to 75 micrometers. Fibrils on and along the acrylic and para-aramid fibrous structures can contact and form a partial cocoon around the rounder, substantially fibril-free, para-aramid particles

The acrylic and para-aramid pulp is without substantial aggregates or conglomerates of the same material. Further, the pulp has a Canadian Standard Freeness (CSF) as measured per TAPPI test T 227 om-92, which is a measure of its drainage characteristics, of 100 to 700 ml, and preferably 250 to 450 ml.

Surface area of pulp is a measure of the degree of fibrillation and influences the porosity of the product made from the pulp. Preferably, the surface area of pulp of this invention is 7 to 11 square meters per gram.

Figure 4 is an image of a photomicrograph of acrylic and para-aramid pulp made according to the process of the present invention.

It is believed that aramid particles and fibrous structures, dispersed substantially homogeneously throughout the reinforcement material, and the friction and sealing materials, provide, by virtue of the high temperature characteristics of the para-aramid polymers and the fibrillation propensity of the para-aramid fibers, many sites of reinforcement and increased wear resistance. When co-refined, the blending of the acrylic and para-aramid materials is so intimate that in a friction or sealing material there is always some para-aramid fibrous structures close to the acrylic structures, so the stresses and abrasion of service are always shared.

### Sealing Material

The invention is further directed to sealing material and processes for making the sealing materials. Sealing materials are used in or as a barrier to prevent the discharge of fluids and/or gases and used to prevent the entrance of contaminants where two items are joined together. An illustrative use for sealing material is in gaskets. The sealing material comprises a binder; optionally at least one filler; and a fibrous reinforcement material comprising the acrylic and para-aramid pulp of this invention. Suitable binders include nitrile rubber, butadiene rubber, neoprene, styrene-butadiene rubber, nitrile-butadiene rubber, and mixtures thereof. The binder can be added with all other starting materials. The binder is typically added in the first step of the gasket production process, in which the dry ingredients are mixed together. Other ingredients optionally include uncured rubber particles and a rubber solvent, or a solution of rubber in solvent, to cause the binder to coat surfaces of the fillers and pulp. Suitable fillers include barium sulfate, clays, talc, and mixtures thereof.

Suitable processes for making sealing materials are, for example, a beater-add process or wet process where the gasket is made from a slurry of materials, or by what is called a calendering or dry process where the ingredients are combined in an elastomeric or rubber solution.

### Friction Material

The pulp of the present invention can be used as a reinforcement material in friction materials. By "friction materials" is meant materials used for their frictional characteristics such as coefficient of friction to stop or transfer energy of motion, stability at high temperatures, wear resistance, noise and vibration damping properties, etc. Illustrative uses for friction materials include brake pads, brake blocks, dry clutch facings, clutch face segments, brake pad backing/insulating layers, automatic transmission papers, and friction papers.

In view of this new use, the invention is further directed to friction material and processes for making the friction material. Specifically, the friction material comprises a friction modifier; optionally at least one filler; a binder; and a fibrous reinforcement material comprising the acrylic and para-aramid pulp of this invention. Suitable friction modifiers are metal powders such as iron, copper and zinc; abrasives such as oxides of magnesium and aluminum; lubricants, such as synthetic and natural graphites, and sulfides of molybdenum and zirconium; and organic friction modifiers such as synthetic rubbers and cashew nut shell resin particles. Suitable binders are thermosetting resins such as phenolic resins (i.e., straight (100%) phenolic resin and various phenolic resins modified with rubber or epoxy), melamine resins, epoxy resins and polyimide resins, and mixtures thereof. Suitable fillers include barite, calcium carbonate, wollastonite, talc, various clays, and mixtures thereof.

The actual steps for making the friction material can vary, depending on the type of friction material desired. For example, methods for making molded friction parts generally involve combining the desired ingredients in a mold, curing the part, and shaping, heat treating and grinding the part if desired. Automotive transmission and friction papers generally can be made by combining the desired ingredients in a slurry and making a paper on a paper machine using conventional paper making processes.

### TEST METHODS

The following test methods were used in the following Examples.

Canadian Standard Freeness (CSF) is a well-known measure of the facility for water to drain from a slurry or dispersion of particles. Freeness is determined by TAPPI test T227. Data obtained from conduct of that test are expressed as Canadian Freeness Numbers, which represent the milliliters of water which drain from an aqueous slurry under specified conditions. A large number indicates a high freeness and a high tendency for water to drain. A low number indicates a tendency for the dispersion to drain slowly. The freeness is inversely related to the degree of fibrillation of the pulp, since greater numbers of fibrils reduce the rate at which water drains through a forming paper mat.

Length-weighted average is measured using a "FiberExpert" tabletop analyzer (also now known as "PulpExpertFS", available from Metso Automation of Helsinki, Finland). This analyzer takes photographic images of the pulp with a digital CCD camera as the pulp slurry flows through the analyzer and then an integrated computer analyzes the fibers in these images and calculates their length-weighted average.

Temperature: All temperatures are measured in degrees Celsius (° C).

Denier is measured according to ASTM D 1577 and is the linear density of a fiber as expressed as weight in grams of 9000 meters of fiber. The denier is measured on a Vibroscope from Textechno of Munich, Germany. Denier times (10/9) is equal to decitex (dtex).

### EXAMPLES

This invention will now be illustrated by the following specific examples. All parts and percentages are by weight unless otherwise indicated. Examples prepared according to the process or processes of the current invention are indicated by numerical values.

### Example 1

In this example of the invention, the pulp of this invention was produced from a feedstock of para-aramid fiber and acrylic staple. Acrylic staple having a cut length of 5 cm (2 inches) and having a filament linear density of 3 dpf (3.3 dtex per filament) was obtained from Solutia, Inc., with offices in St. Louis, MO. Para-aramid fiber in the form of commercially available KEVLAR^{®} brand floc, Style 1 F178, having a %" cut length, was obtained from E. I. de Pont de Nemours and Company with offices in Wilmington, Delaware.

Acrylic staple and water together were fed directly into a Sprout-Waldron 12" Single Disc Refiner using a 10 mil plate gap setting and pre-pulped to reach an acceptable processing length in the range of 13mm.

The pre-pulped acrylic fiber and the cut para-aramid fiber plus water were then combined into a highly agitated mixing tank at a solids concentration of 50 wt % para-aramid fiber and 50 wt% acrylic staple and mixed to form a uniform, pumpable slurry of about 2-3 wt % of the total ingredients concentration The slurry was then recirculated and co-refined through a Sprout-Waldron 12" Single Disc Refiner.

The refiner simultaneously:
(1) fibrillated, cut, and masticated both the para-aramid fiber and the acrylic staple to irregularly shaped fibrous structures having stalks and fibrils.
(2) dispersed all solids such that the refined slurry was substantially uniform, substantially uniform being as previously defined.

This refined slurry was then filtered using a filter bag and was dewatered through pressing and placed in large ZIPLOC^{®} type storage bags. The fibrous structures had an average maximum dimension of no more than 5 mm and a length-weighted average of no more than 1.3 mm, as measured by FiberExpert^{®}.

### Example 2

This example illustrates another method by which a co-refined pulp can be made from a feedstock of para-aramid fiber and acrylic fiber. Acrylic staple, having a cut length of 5 cm (2 inches) and having a filament linear density of 3 dpf (3.3 dtex per filament) available from Solutia, Inc., is cut with a guillotine cutter two to three times at right angles in order to produce a random-length fiber with most fibers shorter than ¾ inch (1.91 cm) and averaging about'/z inch (1.27 cm) long.

Para-aramid fiber in the form of commercially available KEVLAR^{®} brand multifilament yarn, available from E. I. de Pont de Nemours and Company on bobbins, is prepared by cutting the para-aramid yarn to a nominal ½ inch (1.27 cm) cut length on a Lummus Cutter (available from Lummus Industries with offices in Columbus, Georgia). Other KEVLAR^{®} brand para-aramid fiber, which initially is not on bobbins and is of multiple long lengths, is cut by a guillotine cutter two to three times at right angles in order to produce a random-length fiber with most fibers shorter than ¾ inch (1.91 cm) and averaging about ½ inch (1.27 cm) long.

The two ingredients prepared as described above plus water are then combined into a highly agitated mixing tank called a hydrapulper at a solids concentration of 50 wt % para-aramid fiber and 50 wt % acrylic fiber and mixed to form a substantially uniform, pumpable slurry having a total solids concentration of about 2-3 wt % of the total ingredients. The slurry is pumped through a series of three refiners, as described in U.S. Patent 4,472,241. The refiners simultaneously:
(1) fibrillate, cut, and masticate the acrylic fiber and the para-aramid fiber into irregularly shaped fibrous structures having stalks and fibrils; and
(2) disperse all solids such that the refined slurry was substantially uniform with substantially uniform as previously defined.

This refined slurry is then dewatered using a horizontal filter and dried in an oven to a desired moisture content of 50 total wt % for wet pulp. The wet pulp is then packaged into bales by a baler. When measured by FiberExpert^{®}, all of the ingredients in the pulp have a length-weighted average of no more than 1.3 mm.

### Example 3

This example illustrates further process steps and another embodiment of the pulp of this invention. The procedure of Example 2 is followed. However, after the pulp is dewatered on the horizontal filter, the pulp is pressed in a mechanical press to further remove water; and the pulp is then fluffed using a Fluffer (available from Bepex Corporation with offices at Santa Rosa, California) to better separate the pressed wet pulp. The fluffed wet pulp is then dried in an oven to approximately 8 total wt % moisture and is then further processed in an ultra rotor (model IIIA available from Altenburger Machinen Jackering GmbH with offices in Voisterhauser, Germany) such as is disclosed in U.S. Patent 5,084,136 to further fluff and disperse the dried pulp. The dried pulp is then packaged into bales. When measured by FiberExpert^{®}, all of the ingredients in the pulp have a length-weighted average of no more than 1.3 mm.

### Example 4

This example illustrates another embodiment of the pulp of this invention. The process of Example 2 is followed with the exception that one third by weight of the para-aramid fiber is replaced by para-aramid particles. The para-aramid resin particles are prepared by reacting para-phenylenediamine and teraphthaloyl chloride continuously in a screw extruder as is generally disclosed in U.S. Patent 3,884,881, but using N, methyl pyrollidone/calcium chloride as the solvent, producing a crumb-like polymer that precipitates from the solvent. The solvent is extracted, and the polymer crumb washed and dried to a particulate powder of mixed particle size. The para-aramid resin particles are then treated substantially the same as the para-aramid fiber is treated in Example 2. However, the refiner not only refines the fibers but also cuts and/or masticates the para-aramid particles into rounder, substantially fibril-free particles. After dewatering, some of the resulting pulp having a moisture content of 50 total wt percent is then packaged into bales. The remainder of the resulting pulp is further pressed to a moisture content of approximately 8 total wt percent and then fluffed, dispersed, and packaged as in Example 3. When measured by FiberExpert^{®}, all of the ingredients in the pulp have a length-weighted average of no more than 1.3 mm.

### Example 5

Disc brake pads incorporating the pulp of this invention were made in the following manner. Approximately 20 kilograms of a non-asbestos-containing base compound powder comprising a mixture of 7 wt % cashew nut shell resin, 17 wt % inorganic fillers, 21 wt % graphite, coke and lubricants, 18 wt % inorganic abrasives, and 16 wt % soft metals was mixed together for 10 to 20 minutes in a 50-liter Littleford mixer. The mixer had two high-speed choppers with blades of the "stars and bars" configuration and a slower rotating plough.

5 kilograms of the well-blended base compound powder was then combined with the pulp of this invention (a co-refined pulp being 50 wt % para-aramid and 50 wt % acrylic fiber) in an amount of 3.8 wt %, based on the combined weight of the compound powder and the pulp. The pulp was then dispersed in the base compound powder by mixing for an additional 5 to 10 minutes. Once mixed, the resulting brake pad composition had a normal visual appearance with the fiber well dispersed in and completely coated with the base compound powders, with essentially no detectable balling up of the pulp or segregation of any constituents.

The brake pad composition was then poured into a single-cavity steel mold for a front disc brake pad and cold pressed to a standard thickness of about 5/8 inch (16 mm) then removed from the mold to form a pre-formed brake pad having an approximate weight of 200 grams. The pre-form had no excessive spring-back or swelling, and was robust enough to endure normal handling without damage. Twelve replicate pre-forms were made. The pre-forms were then placed in two multi-cavity molds, placed in a commercial press, and press-cured (the binder phenolic cross-linking and reacting) at 300°F (149°C) for about 15 minutes, with periodic pressure release to allow phenolic reaction gases to escape, followed by lightly constrained oven curing at 340°F (171°C) for 4 hours to complete the phenolic binder crosslinking. The cured, molded pad was then ground to the desired thickness of about half an inch (13 mm). When compared visually with a commercial brake pad containing an equivalent amount of all para-aramid pulp or acrylic pulp, the test pad was indistinguishable and had good compound flow into the backing plate holes and no edge chipping.

A sample of the brake pad incorporating the pulp of this invention was then tested to determine its frictional performance. Coupons, typically one inch by one inch and about 3/16 inch (5 mm) thick, from test pads were assessed on the Chase Machine available from Link Engineering, Detroit, MI, using test protocol Society of Automotive Engineers (SAE) J661 to determine the hot and cold friction coefficient during constant pressure and controlled temperature drag tests against a heated steel drum. The sample was periodically measured for wear (thickness loss). This was repeated with two more test samples cut from other replicate pads. The samples of the brake pad incorporating the pulp of this invention exhibited hot and cold friction performance substantially equivalent to commercially available pads containing a substantially equivalent amount of all para-aramid pulp. The test further indicated the pad-to-pad uniformity and an average friction rating was also substantially equivalent.

The pad was then tested for friction and wear under various braking conditions using a dynamometer (single piston dynamometer with a rolling radius of 289.0 mm at Link Testing Laboratories, Inc., in Detroit, MI) using test protocol J2681 (ISO-SWG4). This test was comprised of seventeen scenarios of from 5 to 200 brake applications each, and measured coefficient of friction as a function of applied brake pressure, temperature, braking speed and deceleration rate. This test also had two high-temperature fade sections, during which the brake pad was subjected to increasingly high initial temperatures during constant deceleration, and reached temperatures exceeding 600°C. Wear was measured as the reduction in thickness and weight of the pad at the end of the test (608 brake applications.) Results for the pads made with the compound of this example showed very little fade and what fade there was recovered well (where fade is defined as the loss of friction at the highest temperature brake applications), acceptable coefficient of friction of 0.25 to 0.4 in non-fade sections, absence of pad surface cracking, and acceptable wear rates for both the pad and the rotor.

### Example 6

This example illustrates how the pulp of this invention can be incorporated into a beater-add gasket for sealing applications. Water, rubber, latex, fillers, chemicals, and the pulp of this invention are combined in desired amounts to form a slurry. On a circulating wire sieve (such as a paper machine screen or wire), the slurry is largely drained of its water content, is dried in a heating tunnel, and is vulcanized on heated calender rolls to form a material having a maximum thickness of around 2.0 mm. This material is compressed in a hydraulic press or two-roll calender, which increases the density and improves sealability.

Such beater-add gasket materials generally do not have as good sealability as equivalent compressed-fiber materials and are best suited for moderate-pressure high-temperature applications. Beater-add gaskets find applicability in the making of auxiliary engine gaskets or, after further processing, cylinder head gaskets. For this purpose, the semi-finished product is laminated onto both sides of a spiked metal sheet and is physically fixed in place by the spikes.

### Example 7

This example illustrates how the pulp of this invention can be incorporated into a gasket made by a calendering process. The same ingredients as in Example 6, minus the water, are thoroughly dry mixed together and are then blended with a rubber solution prepared using an appropriate solvent.

After mixing, the compound is then generally conveyed batchwise to a roll calender. The calender consists of a small roll that is cooled and a large roll that is heated. The compound is fed and drawn into the calender nip by the rotary movement of the two rolls. The compound will adhere and wrap itself around the hot lower roll in layers generally about 0.02 mm thick, depending on the pressure, to form a gasketing material made from the built-up compound layers. In so doing, the solvent evaporates and vulcanization of the elastomer commences.

Once the desired gasketing material thickness is reached, the rolls are stopped and the gasketing material is cut from the hot roll and cut and/or punched to the desired size. No additional pressing or heating is required, and the material is ready to perform as a gasket. In this manner gaskets up to about 7 mm thick can be manufactured. However, most gaskets made in this manner are much thinner, normally being about 3 mm or less in thickness.

## Claims

1. A process for making an acrylic and para-aramid pulp for use as reinforcement material, comprising:
(a) combining pulp ingredients including:
(1) acrylic fiber comprising acrylonitrile units which are at least 85 wt % of the total acrylic fiber, the fiber being 10 to 90 wt % of the total solids in the ingredients, and having an average length of no more than 10 cm;
(2) para-aramid fiber being 10 to 90 wt % of the total solids in the ingredients, and having an average length of no more than 10 cm; and
(3) water being 95 to 99 wt % of the total ingredients;
(b) mixing the ingredients to a substantially uniform slurry;
(c) co-refining the slurry by simultaneously:
(1) fibrillating, cutting and masticating the acrylic fiber and the para-aramid fiber to irregularly shaped fibrillated fibrous structures with stalks and fibrils; and
(2) dispersing all solids such that the refined slurry is substantially uniform; and
(d) removing water from the refined slurry to no more than 60 total wt % water,
thereby producing an acrylic and para-aramid pulp with the acrylic and the para-aramid fibrous structures having an average maximum dimension of no more than 5 mm, a length-weighted average of no more than 1.3 mm, and the acrylic fibrils and/or stalks are substantially entangled with the para-aramid fibrils and/or stalks.

2. The process of Claim 1, wherein
the acrylic fiber has a linear density of no more than 10 dtex; and
and the para-aramid fiber has a linear density of no more than 2.5 dtex.

3. The process of Claim 1, wherein the pulp being without substantial aggregates of the same material.

4. The process of Claim 1, wherein
the ingredients further comprise
substantially or completely fibril-free, granular, para-aramid particles being no more than 50 wt % of the total solids in the ingredients, and having an average maximum dimension of 50 to 2000 microns, and
in the refining step, masticating at least some of the para-aramid particles into smaller, rounder, substantially fibril-free, particles,
whereby in the produced acrylic and para-aramid pulp, the acrylic and para-aramid fibrous structures contact and are wrapped partially around at least some of the rounder, substantially fibril-free, para-aramid particles.

5. The process of Claim 1, wherein in the combining step, the acrylic fiber comprises 25 to 60 wt % of the total solids.

6. The process of Claim 1, wherein in the combing step, the para-aramid fiber comprises 40 to 75 wt % of the total solids.

7. The process of Claim 1, wherein after the removing step, the water being 4 to 60 wt % of the entire pulp, and the pulp having a Canadian Standard Freeness (CSF) of 100 to 700 ml.

8. The process of Claim 1, wherein the refining step comprises passing the mixed slurry through a series of disc refiners.

9. A process for making an acrylic and para-aramid pulp for use as reinforcement material, comprising:
(a) combining ingredients including water and a first fiber from the group consisting of:
(1) acrylic fiber comprising acrylonitrile units which are at least 85 wt % of the total acrylic fiber, the fiber being 10 to 90 wt % of the total solids in the pulp; and
(2) para-aramid fiber being 10 to 90 wt % of the total solids in the pulp;
(b) mixing the combined ingredients to a substantially uniform suspension;
(c) refining the suspension in a disc refiner thereby cutting the fiber to have an average length of no more than 10 cm, and fibrillating and masticating at least some of the fiber to irregularly shaped fibrillated fibrous structures;
(d) combining ingredients including the refined suspension, the second fiber of the group of (a)(1 and 2) having an average length of no more than 10 cm, and water, if necessary, to increase the water concentration to 95 -99 wt % of the total ingredients;
(e) mixing the ingredients, if necessary, to form a substantially uniform suspension;
(f) co-refining the mixed suspension by simultaneously:
(1) fibrillating, cutting and masticating solids in the suspension such that all or substantially all of the acrylic and para-aramid fiber is converted to irregularly shaped fibrillated acrylic and para-aramid fibrous structures with stalks and fibrils; and
(2) dispersing all solids such that the refined slurry is substantially uniform; and
(g) removing water from the refined slurry to no more than 60 total wt % water,
thereby producing an acrylic and para-aramid pulp with the acrylic and the para-aramid fibrous structures having an average maximum dimension of no more than 5 mm, a length-weighted average of no more than 1.3 mm, and the acrylic fibrils and/or stalks are substantially entangled with the para-aramid fibrils and/or stalks.

10. The process of Claim 9, wherein
the ingredients further comprise:
substantially or completely fibril-free, granular, para-aramid particles being no more than 50 wt % of the total solids in the ingredients, and having an average maximum length of 50 to 2000 microns; and
in either the first or second refining step, masticating at least some of the para-aramid particles into smaller, rounder, substantially fibril-free, particles,
whereby in the produced acrylic and para-aramid pulp, the acrylic and para-aramid fibrous structures contact and are wrapped partially around at least some of the rounder, substantially fibril-free, para-aramid particles.

11. The process of Claim 9, wherein after the removing step, the irregularly shaped acrylic fibrous structures being 25 to 60 wt % of the total solids.

12. The process of Claim 9, wherein after the removing step, the irregularly shaped, para-aramid, fibrous structures being 40 to 75 wt % of the total solids.

13. The process of Claim 9, wherein after the removing step, the water being 4 to 60 wt % of the entire pulp, and the pulp having a Canadian Standard Freeness (CSF) of 100 to 700 ml.

14. An acrylic and para-aramid pulp for use as reinforcement material, comprising:
(a) irregularly shaped, acrylic fibrous structures comprising acrylonitrile units which are at least 85 wt % of the total acrylic fibrous structures, the structures being 10 to 90 wt % of the total solids;
(b) irregularly shaped, para-aramid fibrous structures being 10 to 90 wt % of the total solids; and
(c) water being 4 to 60 wt % of the entire pulp,
whereby the acrylic and the para-aramid fibrous structures having an average maximum dimension of no more than 5 mm, a length-weighted average of no more than 1.3 mm, and stalks and fibrils where the acrylic fibrils and/or stalks are substantially entangled with the para-aramid fibrils and/or stalks.

15. The aramid pulp of Claim 14, further comprising
substantially or completely fibril-free, granular, para-aramid particles being no more than 50 wt % of the total solids.

16. The pulp of Claim 14, wherein
the irregularly shaped, acrylic fibrous structures being 25 to 60 wt % of the total solids.

17. The pulp of Claim 14, wherein
the irregularly shaped, para-aramid, fibrous structures being 40 to 75 wt % of the total solids.

18. The pulp of Claim 14, wherein the water being 4 to 60 wt % of the entire pulp, and the pulp having a Canadian Standard Freeness (CSF) of 100 to 700 ml.

19. A friction material, comprising:
a friction modifier;
a binder; and
a fibrous reinforcement material comprising the pulp of Claim 14.

20. The friction material of Claim 19, wherein
the friction modifier is selected from the group consisting of metal powders, abrasives, lubricants, organic friction modifiers, and mixtures thereof; and
the binder is selected from the group consisting of thermosetting resins, melamine resins, epoxy resins and polyimide resins, and mixtures thereof.

21. A sealing material, comprising:
a binder; and
a fibrous reinforcement material comprising the pulp of Claim 14.

22. The sealing material of Claim 21, wherein
the binder is selected from the group consisting of nitrile rubber, butadiene rubber, neoprene, styrene butadiene rubber, nitrile-butadiene rubber, and mixtures thereof.

## Patentansprüche

1. Verfahren zum Herstellen einer Acryl- und para-Aramid-Pulpe zur Verwendung als Verstärkungsmaterial, umfassend:
(a) Kombinieren der Pulpenbestandteile, die Folgendes einschließen:
(1) Acryl-Fasern, umfassend Acrylnitril-Einheiten, die mindestens 85Gew.-% der Gesamtacryl-Fasern darstellen, wobei die Fasern 10 bis 90 Gew.-% der Gesamtfeststoffe in den Bestandteilen ausmachen und eine durchschnittliche Länge von nicht mehr als 10 cm aufweisen;
(2) para-Aramid-Fasern, die 10 bis 90 Gew.-% der Gesamtfeststoffe in den Bestandteilen ausmachen und eine durchschnittliche Länge von nicht mehr als 10 cm aufweisen; und
(3) Wasser, das 95 bis 99 Gew.-% der Gesamtbestandteile ausmacht;
(b) Mischen der Bestandteile zu einem im Wesentlichen einheitlichen Brei;
(c) gemeinsames Verfeinern des Breis durch simultanes:
(1) Fibrillieren, Schneiden und Mastizieren der Acryl-Fasern und der para-Aramid-Fasern zu unregelmäßig geformten fibrillierten Faserstrukturen mit Stängeln und Fibrillen; und
(2) Dispergieren aller Feststoffe dergestalt, dass der verfeinerte Brei im Wesentlichen einheitlich ist; und
(d) Entfernen von Wasser aus dem verfeinerten Brei auf nicht mehr als 60 Gew.-% Gesamtwasser,
wodurch eine Acryl- und para-Aramid-Pulpe mit den Acryl- und den para-Aramid-Faserstrukturen hergestellt wird, die eine durchschnittliche maximale Abmessung von nicht mehr als 5 mm, einen längengewichteten Durchschnitt von nicht mehr als 1,3 mm aufweisen, und die Acryl-Fibrillen und/oder -Stängel mit den para-Aramid-Fibrillen und/oder -Stängeln im Wesentlichen verknäult sind.

2. Verfahren nach Anspruch 1, worin
die Acryl-Fasern eine lineare Dichte von nicht mehr als 10 dtex aufweisen; und
die para-Aramid-Fasern eine lineare Dichte von nicht mehr als 2,5 dtex aufweisen.

3. Verfahren nach Anspruch 1, worin die Pulpe ohne wesentliche Aggregate aus dem gleichen Material besteht.

4. Verfahren nach Anspruch 1, worin die Bestandteile weiter Folgendes umfassen:
im Wesentlichen oder vollständig fibrillenfreie, granuläre para-Aramid-Partikel, die nicht mehr als 50 Gew.-% der Gesamtfeststoffe in den Bestandteilen ausmachen und eine durchschnittliche maximale Abmessung von 50 bis 2000 µm aufweisen, und
im Verfeinerungsschritt, Mastizieren von mindestens einigen der para-Aramid-Partikel zu kleineren, runderen, im Wesentlichen fibrillen freien Partikeln,
wobei in der hergestellten Acryl- und para-Aramid-Pulpe die Acryl- und para-Aramid-Faserstrukturen mindestens einige der runderen, im Wesentlichen fibrillenfreien para-Aramid-Partikel kontaktieren und teilweise um sie herumgewickelt sind.

5. Verfahren nach Anspruch 1, worin die Acryl-Fasern im Kombinationsschritt 25 bis 60 Gew.-% der Gesamtfeststoffe umfassen.

6. Verfahren nach Anspruch 1, worin die para-Aramid-Fasern im Kombinationsschritt 40 bis 75 Gew.-% der Gesamtfeststoffe umfassen.

7. Verfahren nach Anspruch 1, worin das Wasser nach dem Entfernungsschritt 4 bis 60 Gew.-% der gesamten Pulpe ausmacht und die Pulpe eine als Canadian Standard Freeness (CSF) angegebene Entwässerungs-"Freiheit" von 100 bis 700 ml aufweist.

8. Verfahren nach Anspruch 1, worin der Verfeinerungsschritt das Durchgeben des gemischten Breis durch eine Reihe von Scheibenrefiner darstellt.

9. Verfahren zum Herstellen einer Acryl- und para-Aramid-Pulpe zur Verwendung als Verstärkungsmaterial, umfassend:
(a) Kombinieren der Bestandteile, einschließlich Wasser und einer ersten Faser aus der Gruppe bestehend aus:
(1) Acryl-Fasern, umfassend Acrylnitril-Einheiten, die mindestens 85 Gew.-% der Gesamtacryl-Fasern darstellen, wobei die Fasern 10 bis 90 Gew.-% der Gesamtfeststoffe in der Pulpe ausmachen; und
(2) para-Aramid-Fasern, die 10 bis 90 Gew.-% der Gesamtfeststoffe in der Pulpe ausmachen;
(b) Mischen der kombinierten Bestandteile zu einer im Wesentlichen einheitlichen Suspension;
(c) Verfeinern der Suspension in einem Scheibenrefiner, wobei die Fasern geschnitten werden, um eine durchschnittliche Länge von nicht mehr als 10 cm aufzuweisen, und Fibrillieren und Mastizieren von mindestens einigen der Fasern zu unregelmäßig geformten fibrillierten Faserstrukturen;
(d) Kombinieren der Bestandteile, einschließlich der verfeinerten Suspension, der zweiten Faser der Gruppe von (a) (1 und 2) mit einer durchschnittlichen Länge von nicht mehr als 10 cm, und gegebenenfalls Wasser zum Steigern der Wasserkonzentration auf 95 - 99 Gew.-% der Gesamtbestandteile;
(e) gegebenenfalls Mischen der Bestandteile zum Bilden einer im Wesentlichen einheitlichen Suspension;
(f) gemeinsames Verfeinern der gemischten Suspension durch simultanes:
(1) Fibrillieren, Schneiden und Mastizieren von Feststoffen in der Suspension dergestalt, dass alle oder im Wesentlichen alle der Acryl- und para-Aramid-Fasern in unregelmäßig geformte fibrillierte Acryl- und para-Aramid-Faserstrukturen mit Stängeln und Fibrillen umgewandelt werden; und
(2) Dispergieren aller Feststoffe dergestalt, dass der verfeinerte Brei im Wesentlichen einheitlich ist; und
(g) Entfernen von Wasser aus dem verfeinerten Brei auf nicht mehr als 60 Gew.-% Wasser insgesamt,
**dadurch** Herstellen einer Acryl- und para-Aramid-Pulpe mit den Acryl- und den para-Aramid-Faserstrukturen, die eine durchschnittliche maximale Abmessung von nicht mehr als 5 mm und einen längegewichteten Durchschnitt von nicht mehr als 1,3 mm aufweisen, und die Acryl-Fibrillen und/oder -Stängel im Wesentlichen mit den para-Aramid-Fibrillen und/oder -Stängeln verknäult sind.

10. Verfahren nach Anspruch 9, worin die Bestandteile weiter Folgendes umfassen:
im Wesentlichen oder vollständig fibrillenfreie, granuläre para-Aramid-Partikel, die nicht mehr als 50 Gew.-% der Gesamtfeststoffe in den Bestandteilen ausmachen und eine durchschnittliche maximale Länge von 50 bis 2000 um aufweisen; und
entweder im ersten oder zweiten Verfeinerungsschritt, Mastizieren von mindestens einigen der para-Aramid-Partikel zu kleineren, runderen, im Wesentlichen fibrillenfreien Partikeln,
wobei in der hergestellten Acryl- und para-Aramid-Pulpe, die Acryl- und para-Aramid-Faserstrukturen mindestens einige der runderen, im Wesentlichen fibrillenfreien para-Aramid-Partikel kontaktieren und teilweise um sie herumgewickelt sind.

11. Verfahren nach Anspruch 9, worin die unregelmäßig geformten Acryl-Faserstrukturen nach dem Entfernungsschritt 25 bis 60 Gew.-% der Gesamtfeststoffe ausmachen.

12. Verfahren nach Anspruch 9, worin die unregelmäßig geformten Para-Aramid-Faserstrukturen nach dem Entfernungsschritt 40 bis 75 Gew.-% der Gesamtfeststoffe ausmachen.

13. Verfahren nach Anspruch 9, worin das Wasser nach dem Entfernungsschritt 4 bis 60 Gew.-% der gesamten Pulpe ausmacht, und die Pulpe eine als Canadian Standard Freeness (CSF) angegebene Entwässerungs-"Freiheit" von 100 bis 700 ml aufweist.

14. Acryl- und para-Aramid-Pulpe zur Verwendung als Verstärkungsmaterial, umfassend:
(a) unregelmäßig geformte Acryl-Faserstrukturen, umfassend Acrylnitril-Einheiten, welche mindestens 85 Gew.-% der Gesamtacryl-Faserstrukturen ausmachen, wobei die Strukturen 10 bis 90 Gew.-% der Gesamtfeststoffe ausmachen;
(b) unregelmäßig geformte para-Aramid-Faserstrukturen, die 10 bis 90 Gew.% der Gesamtfeststoffe ausmachen; und
(c) Wasser, das 4 bis 60 Gew.-% der gesamten Pulpe ausmacht,
wobei die Acryl- und die para-Aramid-Faserstrukturen Folgendes aufweisen: eine durchschnittliche maximale Abmessung von nicht mehr als 5 mm, einen längengewichteten Durchschnitt von nicht mehr als 1,3 mm, und Stängel und Fibrillen, worin die Acryl-Fibrillen und/oder -Stängel im Wesentlichen mit den para-Aramid-Fibrillen und/oder -Stängeln verknäult sind.

15. Aramidpulpe nach Anspruch 14, weiter umfassend im Wesentlichen oder vollkommen fibrillenfreie, granuläre para-Aramid-Partikel, die nicht mehr als 50 Gew.% der Gesamtfeststoffe ausmachen.

16. Pulpe nach Anspruch 14, worin
die unregelmäßig geformten Acryl-Faserstrukturen 25 bis 60 Gew.- % der Gesamtfeststoffe ausmachen.

17. Pulpe nach Anspruch 14, worin
die unregelmäßig geformten Para-Aramid-Faserstrukturen 40 bis 75 Gew.-% der Gesamtfeststoffe ausmachen.

18. Pulpe nach Anspruch 14, worin das Wasser 4 bis 60 Gew.-% der gesamten Pulpe ausmacht und die Pulpe eine als Canadian Standard Freeness (CSF) angegebene Entwässerungs-"Freiheit" von 100 bis 700 ml aufweist.

19. Friktionsmaterial, umfassend:
ein Friktionsmodifikationsmittel;
ein Bindemittel; und
ein Faserverstärkungsmaterial, umfassend die Pulpe nach Anspruch 14.

20. Friktionsmaterial nach Anspruch 19, worin
das Friktionsmodifikationsmittel aus der Gruppe ausgewählt ist, bestehend aus Metallpulvern, Abrasivmitteln, Gleitmitteln, organischen Friktionsmodifikationsmitteln und Gemischen davon; und
das Bindemittel aus der Gruppe ausgewählt ist, bestehend aus wärmehärtbaren Harzen, Melaminharzen, Epoxidharzen und Polyimidharzen und Gemischen davon.

21. Abdichtungsmaterial, umfassend:
ein Bindemittel; und
ein Faserverstärkungsmaterial, umfassend die Pulpe nach Anspruch 14.

22. Abdichtungsmaterial nach Anspruch 21, worin
das Bindemittel aus der Gruppe ausgewählt ist, bestehend aus Nitril-Kautschuk, Butadien-Kautschuk, Neopren, Styrol-Butadien-Kautschuk, Nitril-Butadien-Kautschuk und Gemischen davon.

## Revendications

1. Procédé de fabrication d'une pâte d'acrylique et para-aramide pour l'utilisation comme matériau de renforcement, comprenant:
(a) la combinaison des ingrédients pour la pâte incluant:
(1) de la fibre acrylique comprenant des motifs d'acrylonitrile qui sont au moins de 85 % en pds de la fibre acrylique totale, la fibre étant de 10 à 90 % en pds des matières solides totales dans les ingrédients, et ayant une longueur moyenne de pas plus de 10 cm;
(2) de la fibre de para-aramide étant de 10 à 90 % en pds des matières solides totales dans les ingrédients, et ayant une longueur moyenne de pas plus de 10 cm; et
(3) de l'eau étant de 95 à 99 % en pds des ingrédients totaux;
(b) le mélange des ingrédients jusqu'à l'obtention d'une suspension substantiellement uniforme;
(c) le co-raffinage de la suspension en simultanément:
(1) fibrillant, découpant et mastiquant la fibre acrylique et la fibre de para-aramide en structures fibreuses fibrillées de forme irrégulière avec des tiges et des fibrilles; et
(2) dispersant toutes les matières solides de sorte que la suspension raffinée soit substantiellement uniforme; et
(d) l'élimination de l'eau de la suspension raffinée jusqu'à pas plus de 60 % en pds totaux d'eau,
produisant de là une pâte d'acrylique et para-aramide avec les structures fibreuses d'acrylique et de para-aramide ayant une dimension maximale moyenne de pas plus de 5 mm, une moyenne pondérée dans la longueur de pas plus de 1,3 mm, et les fibrilles et/ou les tiges d'acryliques sont substantiellement entremêlées avec les fibrilles et/ou les tiges de para-aramide.

2. Procédé selon la revendication 1, dans lequel
la fibre acrylique a une densité linéaire de pas plus de 10 dtex; et
la fibre de para-aramide a une densité linéaire de pas plus de 2,5 dtex.

3. Procédé selon la revendication 1, dans lequel la pâte se trouve sans agrégats substantiels du même matériau.

4. Procédé selon la revendication 1, dans lequel
les ingrédients comprennent en outre des particules de para-aramide, granuleuses, substantiellement ou complètement exemptes de fibrilles étant de pas plus de 50 % en pds des matières solides totales dans les ingrédients, et ayant une dimension maximale moyenne de 50 à 2000 microns, et
dans l'étape de raffinage, la mastication d'au moins une partie des particules de para-aramide en particules plus petites, plus rondes, substantiellement exemptes de fibrilles,
moyennant quoi dans la pâte d'acrylique et para-aramide produite, les structures fibreuses d'acrylique et de para-aramide entrent en contact et sont enveloppées partiellement autour d'au moins une partie des particules de para-aramide plus rondes, substantiellement exemptes de fibrilles.

5. Procédé selon la revendication 1, dans lequel dans l'étape de combinaison, la fibre d'acrylique comprend 25 à 60 % en pds de matières solides totales.

6. Procédé selon la revendication 1, dans lequel dans l'étape de combinaison, la fibre de para-aramide comprend 40 à 75 % en pds de matières solides totales.

7. Procédé selon la revendication 1, dans lequel après l'étape d'élimination, l'eau étant de 4 à 60 % en pds de la pâte entière, et la pâte ayant un indice canadien d'égouttage (CSF) de 100 à 700 ml.

8. Procédé selon la revendication 1, dans lequel l'étape de raffinage comprend le fait de faire passer la suspension mixte à travers une série de raffineurs à disque.

9. Procédé de fabrication d'une pâte d'acrylique et para-aramide pour l'utilisation comme matériau de renforcement, comprenant:
(a) la combinaison des ingrédients incluant l'eau et une première fibre à partir du groupe constitué de:
(1) fibre acrylique comprenant des motifs d'acrylonitrile qui sont d'au moins 85 % en pds de la fibre acrylique totale, la fibre étant de 10 à 90 % en pds des matières solides totales dans la pâte; et
(2) fibre de para-aramide étant de 10 à 90 % en pds des matières solides totales dans la pâte;
(b) le mélange des ingrédients combinés jusqu'à l'obtention d'une suspension substantiellement uniforme;
(c) le raffinage de la suspension dans un raffineur à disque découpant de là la fibre pour avoir une longueur moyenne de pas plus de 10 cm, et la fribrillation et la mastication d'au moins une partie de la fibre jusqu'à des structures fibreuses fibrillées de forme irrégulière;
(d) la combinaison des ingrédients incluant la suspension raffinée, la seconde fibre du groupe de (a) (1 et 2) ayant une longueur moyenne de pas plus de 10 cm, et de l'eau, si nécessaire, pour augmenter la concentration de l'eau jusqu'à 95 à 99 % en pds des ingrédients totaux;
(e) le mélange des ingrédients, si nécessaire, pour former une suspension substantiellement uniforme;
(f) le co-raffinage de la suspension mixte en simultanément:
(1) fibrillant, découpant et mastiquant les matières solides dans la suspension de sorte que toute ou substantiellement toute la fibre d'acrylique et para-aramide soit convertie en structures fibreuses d'acrylique et de para-aramide fibrillées de forme irrégulière avec des tiges et des fibrilles; et
(2) dispersant toutes les matières solides de sorte que la suspension raffinée soit substantiellement uniforme; et
(g) l'élimination de l'eau de la suspension raffinée jusqu'à pas plus de 60 % en pds d'eau au total,
produisant de là une pâte d'acrylique et para-aramide avec les structures fibreuses d'acrylique et de para-aramide ayant une dimension maximale moyenne de pas plus de 5 mm, une moyenne pondérée dans la longueur de pas plus de 1,3 mm, et les fibrilles et/ou les tiges d'acrylique sont substantiellement entremêlées avec les fibrilles et/ou les tiges de para-aramide.

10. Procédé selon la revendication 9, dans lequel
les ingrédients comprennent en outre:
des particules de para-aramide, granuleuses, substantiellement ou complètement exemptes de fibrilles étant de pas plus de 50 % en pds des matières solides totales dans les ingrédients, et ayant une longueur maximale moyenne de 50 à 2000 microns; et
dans soit la première soit la seconde étape de raffinage, la mastication d'au moins une partie des particules de para-aramide en particules plus petites, plus rondes, substantiellement exemptes de fibrilles,
moyennant quoi dans la pâte d'acrylique et para-aramide produite, les structures fibreuses d'acrylique et de para-aramide entrent en contact et sont enveloppées partiellement autour d'au moins une partie des particules de para-aramide plus rondes, substantiellement exemptes de fibrilles.

11. Procédé selon la revendication 9, dans lequel après l'étape d'élimination, les structures fibreuses d'acrylique de forme irrégulière étant de 25 à 60 % en pds des matières solides totales.

12. Procédé selon la revendication 9, dans lequel après l'étape d'élimination, les structures fibreuses et de para-aramide de forme irrégulière étant de 40 à 75 % en pds des matières solides totales.

13. Procédé selon la revendication 9, dans lequel après l'étape d'élimination, l'eau étant de 4 à 60 % en pds de la pâte entière, et la pâte ayant un indice canadien d'égouttage (CSF) de 100 à 700 ml.

14. Pâte d'acrylique et para-aramide pour l'utilisation comme matériau de renforcement, comprenant:
(a) des structures fibreuses d'acrylique de forme irrégulière comprenant des motifs d'acrylonitrile qui sont d'au moins 85 % en pds des structures fibreuses acryliques totales, les structures étant de 10 à 90 % en pds des matières solides totales;
(b) des structures fibreuses de para-aramide, de forme irrégulière étant de 10 à 90 % en pds des matières solides totales; et
(c) de l'eau étant de 4 à 60 % en pds de la pâte entière,
moyennant quoi les structures fibreuses d'acrylique et de para-aramide ayant une dimension maximale moyenne de pas plus de 5 mm, une moyenne pondérée dans la longueur de pas plus de 1,3 mm, et des tiges et des fibrilles où les fibrilles et/ou les tiges d'acrylique sont substantiellement entremêlées avec les fibrilles et/ou les tiges de para-aramide.

15. Pâte d'aramide selon la revendication 14, comprenant en outre
des particules de para-aramide, granuleuses, substantiellement ou complètement exemptes de fibrilles étant de pas plus de 50 % en pds des matières solides totales.

16. Pâte selon la revendication 14, dans laquelle
les structures fibreuses d'acrylique de forme irrégulière étant de 25 à 60 % en pds des matières solides totales.

17. Pâte selon la revendication 14, dans laquelle
les structures fibreuses de para-aramide, de forme irrégulière étant de 40 à 75 % en pds des matières solides totales.

18. Pâte selon la revendication 14, dans laquelle l'eau étant de 4 à 60 % en pds de la pâte entière, et la pâte ayant un indice canadien d'égouttage (CSF) de 100 à 700 ml.

19. Matériau de friction, comprenant:
un agent de modification de la friction;
un liant; et
un matériau de renforcement fibreux comprenant la pâte selon la revendication 14.

20. Matériau de friction selon la revendication 19, dans lequel
l'agent de modification de la friction est choisi parmi le groupe constitué des poudres métalliques, des abrasifs, des lubrifiants, des agents organiques de modification de la friction, et des mélanges de ceux-ci; et
le liant est choisi parmi le groupe constitué des résines thermodurcissables, des résines de type mélamine, des résines époxy et des résines de type polyimide, et des mélanges de celles-ci.

21. Matériau d'étanchéité, comprenant:
un liant; et
un matériau de renforcement fibreux comprenant la pâte selon la revendication 14.

22. Matériau d'étanchéité selon la revendication 21, dans lequel
le liant est choisi parmi le groupe constitué du caoutchouc de nitrile, du caoutchouc de butadiène, du néoprène, du caoutchouc de styrène-butadiène, du caoutchouc de nitrile-butadiène, et des mélanges de ceux-ci.
